

## UNITED STATES PATENT OFFICE

GEORGE A. RICHTER, OF BERLIN, NEW HAMPSHIRE, ASSIGNOR TO BROWN COMPANY, OF BERLIN, NEW HAMPSHIRE, A CORPORATION OF MAINE

## ARTIFICIAL LEATHER AND PROCESS OF MANUFACTURING SAME

No Drawing. Application filed March 16, 1927, Serial No. 175,946. Renewed October 25, 1932.

In manufacturing artificial leather and like materials, it is common practice to impregnate a textile fabric base or foundation with rubber latex or a rubber solution, then to fix 5 the rubber in the fabric by evaporation of the liquid vehicle or solvent, and finally, if desired, to vulcanize the impregnated fabric. In like manner, it has also been proposed to impregnate paper or interfelted fibrous 10 foundations. But interfelted foundation or base material comprising relatively short fibers, as heretofore made, has been found unsatisfactory for the production of artificial leather, doubtless because such short-fibered 15 material, which is initially considerably weaker than a textile, is incapable of absorbing sufficient rubber to impart the necessary body, strength, tear resistance and elasticity of artificial leather; and even the so-called 20 paper felts prepared from cotton or wool fiber, or strong papers prepared from manila, or rope fiber, or so-called sulphate pulp, are of insufficient strength and absorptivity to produce a good artificial leather having optimum characteristics of weight, tear resistance, etc.

I have found that a paper web in which fibers, such as hereinafter described, exist in interfelted but in uncompactated, loose condition, is so highly absorptive that, notwithstanding its lack of initial tensile strength, it constitutes an excellent base or foundation material for the manufacture of artificial leather. Such a paper web is preferably formed of unbeaten or very lightly beaten fiber, as its absorptive capacity is greater when its fibers are unhydrated. By beaten fiber, I mean fiber which has been beaten or hydrated to produce a relatively slow stock 35 in which the individual fibers are more or less coated with cellulose hydrate or gel, and not wood pulp or the like in the form as ordinarily purchased, which has merely been disintegrated or individualized in a beater engine.

A paper web such as herein desired is formed by felting the unbeaten or lightly beaten fiber on a papermaking machine, and removing water therefrom, preferably without 40 compacting its fibers by subjecting it to

heavy suction or to mechanical pressure devices, such as squeeze rolls. Such a paper web is thus formed under conditions different from those maintained during usual paper manufacture, wherein the wet paper web is 55 dewatered as much as possible prior to drying by heavy suction and by press rolls, and is then subjected during drying to the pressure of the drier felts against the drier rolls. Even in the manufacture of so-called hand- 60 made papers, the sheets after formation on the hand mould are subjected to substantial couching pressures when removed, and subjected to pressure during drying, as it is desirable that sufficient pressure be exerted 65 to produce a compact paper.

In forming an absorptive paper web, such as herein desired, the usual papermaking machines, e. g., a machine of the Fourdrinier type, may be employed, but the web is formed and allowed to remain on the moving wire until it is substantially dried; or, after partial dewatering, it may be transferred to another moving wire, upon which it is dried. For instance, after the web is formed, it may 70 be partially dewatered by passing it over one or more suction boxes or rolls maintained under light suction, but it is preferably not subjected to any mechanical pressure devices. While still on the wire, it is dried, as by passing it over a series of hot plates or over a series of drying rolls, preferably without undergoing mechanical compacting during 75 such drying.

If desired, the absorptivity of the web, 80 preferably while dry, may further be increased by wetting or saturating the web with a suitable surface-tension-reducing reagent, such as methyl or ethyl alcohols, acetone, soap solution, or the like, and then drying it. The web initially swells or expands when wetted with such reagents, but undergoes little shrinkage or contraction on drying, as such reagents are removed without exerting as high a surface tension on the 85 fiber as when water alone is used.

The resulting dry paper web is highly 90 bulbous and absorptive, as its interfelted fibers exist in an uncompactated and loose and more or less fluffy condition. Such a web 95 100

is not only absorptive in consequence of the large voids or interstices between the fibers, but also in consequence of the unbeaten condition of the fibers, which prevents material 5 shrinking. Thus, whereas a web formed of hydrated or beaten fiber, upon drying, shrinks considerably and the cellulose hydrate on hardening fills the pores and cells of the web, a web formed of very free stock, 10 as herein described, shrinks but little and is highly porous and absorptive.

In preparing a bibulous web such as described, I preferably use a high alpha cellulose-containing wood fiber, i. e., one which 15 has a high proportion of alpha cellulose and is substantially free from oxy cellulose and other non-alpha cellulosic components. Such fiber is prepared by extracting or dissolving the non-alpha cellulosic material 20 from chemical wood pulp (derived from the digestion of wood chips), by a series of treatments with chemical reagents without appreciably degrading the alpha cellulose content of such pulp, as disclosed in patent 25 application, Serial No. 716,154, filed May 27, 1924, by Milton O. Schur and myself. Preferably, an alpha fiber derived from kraft pulp as described in my application, Serial No. 73,193, filed December 4, 1925, is employed, as such fiber not only possesses high 30 absorbency, but possesses high strength and tear resistance, doubtless because of its long average fiber length. As disclosed in both the afore-mentioned applications, the pre- 35 liberated or chemical wood pulp is refined in an alkaline liquor to higher alpha cellulose content, namely, an alpha cellulose content of at least about 93%. The high absorptive capacity of such alpha pulp is doubtless a 40 consequence of the highly cellular or porous structure of the individual fibers, as a result of the extraction of the impurities or non-alpha cellulose constituents from the fiber cells. A certain proportion of mercerized 45 fiber, which may be alpha or other fiber, may be incorporated in desired proportion into the web-forming stock. The presence of such fiber is advantageous, as it is bulky and absorbent; and a web formed from such fiber 50 undergoes very low shrinkage upon drying. Preferably, however, it is not used alone, as it does not readily form or interfelt by itself into a web of uniform texture on papermaking machines.

55 The dry, bibulous web produced as hereinbefore described may be readily impregnated with rubber by proper treatment. In one case, this is accomplished by passing the web through an aqueous rubber dispersion either 60 in the form of natural rubber latex or in the form of an artificial dispersion or latex prepared from crude or reclaimed rubber. The dispersion may contain, say from 10% to 30% rubber, and may also contain a suitable proportion, say, 2% to 5% of sulphur or its

equivalent when it is desired to produce a vulcanized product. Also, if desired, accelerators of vulcanization, fillers, pigments, resins, or other compounds may be added to the dispersion in such proportion as will result in a product of the desired characteristics. In passing through the dispersion, the web becomes thoroughly soaked or impregnated therewith, whereupon it is passed through rolls which serve to remove only excess dispersion therefrom, without effecting an appreciable compacting of the web, the resulting rubber-dispersion-impregnated web being of the desired rubber content. The water of the dispersion may be removed by evaporation; or the web may be passed through a suitable coagulating medium, say, an acetic acid solution of 5% to 10% concentration, or through a coagulating atmosphere, such as acetic acid vapors, sulphur dioxide, or the like. Preferably, a coagulating atmosphere is employed, as the coagulating vapor or gas penetrates the web more easily to yield a more uniformly permeated product and serves to coagulate and fix the rubber more satisfactorily on the fibers in the web. The greater uniformity of the product is due to the fact that by coagulating the rubber before drying, migration of the dispersed rubber particles along with the water to the surface of the web, where evaporation takes place during subsequent drying, is avoided. Such migration is especially serious when the usual alkali-preserved latex of commerce or the usual artificial latices or dispersions are used in association with a highly bibulous web such as herein described, in which the capillary action is especially high. In any event, however, the dispersed rubber is preferably coagulated in situ in the voids and on the fibers to produce a web permeated with coagulated rubber before drying. The resulting product has excellent so-called "ply adhesion," or tenacity of bond between its face portions or layers, high resistance being encountered to the pulling apart of the dried product after it has been split. If, on the other hand, considerable migration of rubber to the surface of the web takes place during drying, the center of the web is left relatively poorer in rubber and the web may easily be pulled apart after splitting. The web is then dried, as by passing it over hot rolls, or through a hot air tunnel. The impregnated web may be dried without previous coagulation of the dispersed rubber therein, depending on the condition of the dispersed rubber component of the dispersion, that is, upon the tendency of the rubber particles to migrate during drying. Inasmuch, however, as coagulation of the dispersion in the web prior to drying apparently effects a more intimate and tenacious bonding together of the fibers, coagulation is preferably effected prior to drying.

If an artificial leather having rigidity or

firmness is desired, the rubber-impregnated web is subjected to vulcanization. The vulcanizing agent may be added to the aqueous rubber dispersion, as stated; and the rubber-  
5 impregnated web containing the vulcanizing agent may be dried at a sufficiently elevated temperature for a sufficient period to produce the desired vulcanization. In other cases, in lieu of incorporating the vulcanizing agent  
10 into the rubber dispersion, vulcanization may be accomplished by passing the rubber-impregnated web through a vulcanizing atmosphere,—for instance, through an atmosphere of sulphur chloride vapors or through  
15 a vulcanizing solution, such as a solution of sulphur chloride in alcohol or carbon bisulphide, or through an atmosphere of hydrogen sulphide or one of sulphur dioxide, or successively through both atmospheres in the order  
20 stated, or in reverse order, with or without the application of heat.

In lieu of an aqueous rubber dispersion as the impregnating medium, a solution of rubber in a suitable solvent, for instance a rubber-  
25 benzol solution of, say, 5% to 10% rubber content, may be used for such purpose. After impregnating the web and removing any excess solution therefrom, its solvent content may be evaporated and recovered.

30 When it is desired to produce a multi-ply artificial leather, a plurality of webs may be simultaneously impregnated with rubber dispersion and then superposed and united as by press-rolls prior to drying, but it is preferable  
35 first to coagulate the rubber and then dry, since by passing the multi-ply web through a coagulating medium, a firm cohesion or bonding together of the contacting faces of the webs by the coagulated rubber is brought  
40 about. If the webs have been impregnated with a rubber solution, their union into a multi-ply web is effected before their solvent content is removed.

The important advantage in employing a  
45 bibulous, uncompacted web formed of alpha fiber such as hereinbefore described is that the artificial leather product realized therefrom may have a rubber content of 100% or greater, based on the dry weight of the web fiber, and  
50 yet simulate natural leather in its appearance, feel and other important physical qualities. Such one is markedly dissimilar to a product wherein a paper web, manufactured by usual methods, serves as a foundation. For instance, the usual blotting paper is far less absorptive than the web herein employed as a foundation and does not in other respects answer the purpose of the present invention. Similarly, a web which is open or porous owing to a loose or "wild" felting on a paper machine, but which has been compacted in the course of its manufacture, does not yield the artificial leather product herein desired, even when made of relatively long fibers, for it  
65 does not possess the absorptivity and other

qualities of a substantially uncompacted web, especially one made of the refined wood pulps hereinbefore described. An uncompacted web may be made from fiber of the order of length of wood fiber derived from spruce, for  
70 example, and yet possess, the absorptivity requisite for the production of the artificial leather product of the present invention.

I present herein a table showing some characteristics of the uncompacted, loosely felted web which I employ, as compared with blotting and with a loosely felted or wild, waterleaf paper composed of relatively long fibers but which has been compacted in the course of its manufacture. The web employed in  
75 producing the product of the present invention was formed of a high alpha cellulose wood fiber prepared from sulphite spruce fiber.

|                         | Waterleaf<br>paper<br>loosely<br>felted<br>but com-<br>pacted | Blotting<br>desk<br>blotter | Paper<br>hard<br>blotter | Alpha<br>fiber<br>web of<br>present<br>invention | 85 |
|-------------------------|---------------------------------------------------------------|-----------------------------|--------------------------|--------------------------------------------------|----|
| Basis weight.....       | 21.4                                                          | 232.0                       | 211.0                    | 24.1                                             | 90 |
| Thickness (inches)..... | .0034                                                         | .0260                       | .0225                    | .0090                                            |    |
| Compactness.....        | 63                                                            | 89                          | 94                       | 27                                               |    |
| Absorptivity.....       | 90 to 150                                                     | 180                         | 130                      | 500 exten-<br>polated,<br>300 in 1.5<br>min.     | 95 |

The compactness value hereinbefore given is obtained by dividing the basis weight by the bulk or thickness in inches, and multiplying by the factor  $10^{-2}$ . The absorptivity was ascertained by noting the water crawl up a strip, the values given denoting hundredths inches crawl up the strip in five minutes. It is to be observed that the compactness of the web used in the product of the present invention is far less, and that its absorptivity is far greater, than that of the other papers compacted as usual in paper-making operations.

Owing to the lack of a better generic expression, the expression rubber-carrying vehicle as used in the appended claims is intended to include the liquid vehicle natural rubber latex, artificial aqueous rubber dispersions, and solutions of rubber in organic solvents, and accordingly by the term "solvent" I mean to include the aqueous phase of a rubber dispersion and also the organic solvent of solutions of rubber.

It do not herein claim the bibulous web per se, or the method of its manufacture, as this constitutes no part of the present invention.

What I claim is:

1. An article of manufacture, comprising a loosely felted, uncompacted paper web of a high alpha cellulose-containing wood fiber permeated with rubber.

2. A process which comprises saturating a loosely felted, uncompacted paper web of wood fiber with rubber latex, and coagulating the rubber in situ within the web by con-

tact with a gaseous coagulating atmosphere.

3. A process which comprises saturating a loosely felted, uncompacted paper web of wood fiber with rubber latex, coagulating the 5 rubber in situ within the web by contact with a gaseous coagulating atmosphere, and drying and vulcanizing the web.

4. A process which comprises forming a 10 cellulosic fibrous paper web in which the fibers exist in a loosely felted, uncompacted condition, saturating said web with acetone, evaporating the acetone, permeating the web with rubber, and vulcanizing the rubber-permeated web.

15 5. As an article of manufacture, a web of interfelted cellulose fiber, at least a portion of which is mercerized, impregnated with rubber.

6. As an article of manufacture, a web of 20 loosely felted, uncompacted cellulose fiber, at least a portion of which is mercerized, impregnated with rubber.

25 7. A process which comprises impregnating a bibulous web of fiber with rubber latex, coagulating the rubber in situ in the web by contact with fumes of acetic acid, and drying the web.

8. A process which comprises impregnating a bibulous web of fiber with rubber latex, 30 coagulating the rubber in situ in the web by contact with sulphur dioxide, and drying the web.

35 9. A process which comprises impregnating a bibulous web of interfelted cellulose fiber with a volatilizable liquid having a much lower surface tension than water alone to swell said web and drying the web to remove said liquid under said lower surface tension and thereby to enhance the porosity 40 of said web.

45 10. A process which comprises impregnating a bibulous web of interfelted cellulose fiber with a volatilizable liquid having a much lower surface tension than water alone to swell said web, drying the web to remove 50 said liquid under said lower surface tension and thereby to enhance the porosity of said web, impregnating the dry web with a rubber-carrying vehicle of a liquid nature, and removing the vehicle.

11. As an article of manufacture, a rubber-impregnated, loosely felted fibrous web, comprising refined wood pulp having an alpha cellulose content of at least about 93%.

55 12. As an article of manufacture, a rubber-impregnated, felted fibrous web comprising substantially unhydrated, refined wood pulp having an alpha cellulose content of at least about 93%.

60 13. A process which comprises refining preliberated cellulose pulp in an alkaline liquor to higher alpha cellulose content, forming a waterlaid, absorptive felt from a furnish containing such refined pulp in a 65 substantially unhydrated condition, impreg-

nating the felt with a rubber-carrying liquid vehicle, and drying the impregnated felt.

70 14. A process which comprises refining preliberated chemical wood pulp in an alkaline liquor to a higher alpha cellulose content, forming a waterlaid, absorptive felt from a furnish containing such refined wood pulp in a substantially unhydrated condition, impregnating the felt with latex, and drying the impregnated felt.

75 15. A process which comprises refining preliberated chemical wood pulp in an alkaline liquor to an alpha cellulose content of at least about 93%, forming a waterlaid, absorptive felt from a furnish containing such refined wood pulp, impregnating the felt with a rubber-carrying liquid vehicle, and drying the impregnated felt.

80 16. A process which comprises refining preliberated chemical wood pulp in an alkaline liquor to an alpha cellulose content of at least about 93%, forming a waterlaid, absorptive felt from a furnish containing such refined wood pulp in a substantially unhydrated condition, impregnating the felt with latex, and drying the impregnated felt.

85 17. A process which comprises forming a felt from a fiber furnish containing mercerized cellulose pulp, impregnating the felt with a rubber-carrying liquid vehicle, and drying the impregnated felt.

90 18. A process which comprises forming a waterlaid felt from a fiber furnish containing mercerized wood pulp, impregnating the felt with latex, and drying the impregnated felt.

95 In testimony whereof I have affixed my signature.

GEORGE A. RICHTER.

105

110

115

120

125

130